

[54] SILVER HALIDE EMULSIONS  
CONTAINING LATENT IMAGE  
STABILIZING COMPOUNDS

[75] Inventor: Arthur H. Herz, Rochester, N.Y.

[73] Assignee: Eastman Kodak Company,  
Rochester, N.Y.

[21] Appl. No.: 236,360

[22] Filed: Feb. 20, 1981

[51] Int. Cl.<sup>3</sup> ..... G03C 1/06

[52] U.S. Cl. ..... 430/505; 430/611;  
430/551

[58] Field of Search ..... 430/611, 505, 551

[56] References Cited

U.S. PATENT DOCUMENTS

|                    |                     |         |
|--------------------|---------------------|---------|
| Re. 28,668 12/1975 | Herz et al. ....    | 430/611 |
| 2,131,038 10/1936  | Brooker et al. .... | 430/614 |
| 3,732,103 5/1973   | Herz et al. ....    | 430/611 |
| 3,824,103 7/1974   | Pierce ....         | 430/611 |
| 3,856,520 12/1974  | Bloom et al. ....   | 430/611 |
| 3,954,478 5/1976   | Arai et al. ....    | 430/551 |

FOREIGN PATENT DOCUMENTS

522997 7/1940 United Kingdom

OTHER PUBLICATIONS

Mills et al., *J. Chem. Soc.*, 123, 2353-2362 (1923).

Williams et al., *J. Amer. Chem. Soc.*, 57, 1856-1876 (1935).

Primary Examiner—John E. Kittle

Assistant Examiner—John L. Goodrow

Attorney, Agent, or Firm—Carl O. Thomas

[57]

ABSTRACT

Photographic silver halide emulsions are protected against latent image fading by latent image stabilizing compounds having the structure:



wherein:

R<sup>1</sup> is hydrogen, alkyl, or aryl;

R<sup>2</sup> and R<sup>3</sup> are each individually hydrogen, alkyl, alkoxyl, carboxyl, alkoxy carbonyl, or aminocarbonyl;

R<sup>4</sup> and R<sup>5</sup> are each individually hydrogen, alkyl, aryl, cyano, halogen, formyl, carboxyl, alkoxy carbonyl, aryloxycarbonyl or aminocarbonyl;

n is an integer of 1 or 2; and

M<sup>⊕n</sup> is a cation of valence n.

18 Claims, No Drawings

## SILVER HALIDE EMULSIONS CONTAINING LATENT IMAGE STABILIZING COMPOUNDS

This invention relates to photographic silver halide emulsions stabilized against latent image fading, to processes of preparing such emulsions and to photographic elements containing them.

A visible image is formed in silver halide photographic materials by exposure of the material to actinic radiation to form a record of the exposure which is invisible to the unaided eye, followed by processing of the material to yield a visible image.

The invisible record of exposure is referred to as a latent image. It is generally agreed that the latent image comprises minute specks of metallic silver formed in or on individual silver halide grains by interaction between silver ions and photoelectrons generated by absorption of actinic radiation by the silver halide grains.

Processing of most common silver halide photographic materials includes a development step in which the material is contacted with an aqueous alkaline solution of a developing agent. The developing agent is a reducing agent which will selectively reduce to metallic silver those silver halide grains containing a latent image.

It is known that the latent image is not permanent and that, with the passage of time, silver halide grains which would be developable immediately after exposure become nondevelopable. This phenomenon is termed latent image fading and manifests itself as a loss in image density in the developed image and a consequent loss in speed in the silver halide photographic material.

If silver halide materials were developed immediately following imagewise exposure, latent image fading would not be a problem. However, with many silver halide materials delays between exposure and processing frequently occur. For example, with amateur film materials in which multiple images are formed on a single roll of film there is often a delay of months between the time the first image is exposed and the time the exposed roll of film is sent for processing. With such materials latent image fading can present a significant problem and compounds are added to photographic materials to prevent or reduce it. These compounds are referred to as latent image stabilizing compounds or latent image stabilizers and the prevention or reduction of latent image fading is referred to as latent image stabilization.

Another way in which the developed image can be adversely affected is through a phenomenon known as fogging. Fogging is a result of spontaneous development of unexposed silver halide grains. The grains can be rendered developable during storage, either prior to or subsequent to exposure, or during development itself. In order to minimize this spontaneous development, compounds known as antifoggants are added to the silver halide material, to the developer solution, or to both.

Some compounds used as antifoggants are structurally similar to compounds used as latent image stabilizers. However, it is important to recognize that the two types of compounds are employed for different purposes to obtain different effects. Latent image fading is the loss of developable silver halide grains and results in a loss in density in the developed silver image, while fogging is the development of unexposed silver halide grains and results in an increase in minimum density.

Thus, compounds which are known to be useful antifoggants are not necessarily useful as latent image stabilizers, and vice versa.

Among the latent image stabilizers known in the art are the N-alkenyl benzothiazolium and naphthothiazolium salts described in Arai et al. U.S. Pat. No. 3,954,478. This patent refers to British Pat. No. 522,997 as showing structurally similar compounds as useful antifoggants, wherein the compounds contain an N-alkyl group rather than an N-alkenyl group. British Pat. No. 522,997 describes, in addition to N-alkyl benzothiazoles and naphthothiazoles, N-alkyl thiiazoles as useful antifoggants. Since Arai et al. were aware of British Pat. No. 522,997, yet described only the N-alkenyl benzothiazolium and naphthothiazolium salts as latent image stabilizers, an inference which can be drawn is that Arai et al. found that the N-alkenyl thiiazolium salts were ineffective as latent image stabilizers. I have confirmed that this is the case. However, I have surprisingly found that acyclic compounds, which can be obtained by basic hydrolysis of N-alkenyl thiiazolium salts, are effective latent image stabilizers.

In accordance with one embodiment of this invention there are provided novel latent image stabilizers represented by the structural formula:



wherein:

$\text{R}^1$  is hydrogen, alkyl, or aryl;

$\text{R}^2$  and  $\text{R}^3$  are each individually hydrogen, alkyl, alkoxy, carboxy, alkoxy carbonyl, or aminocarbonyl;

$\text{R}^4$  and  $\text{R}^5$  are each individually hydrogen, alkyl, aryl, cyano, halogen, formyl, carboxy, alkyl carbonyl, aryl carbonyl, alkoxy carbonyl, aryloxy carbonyl or aminocarbonyl;

$n$  is an integer of 1 or 2; and

$\text{M}^{\oplus n}$  is a cation of valence  $n$ .

The alkyl groups and the alkyl portions of the alkoxy, alkyl carbonyl and alkoxy carbonyl groups preferably contain 1 to 8 carbon atoms (e.g., methyl, ethyl, propyl, butyl, amyl, hexyl, octyl), and most preferably contain 1 to 4 carbon atoms, and include unsubstituted and substituted groups. Useful substituents include halogen, cyano, aryl, carboxy, alkyl carbonyl, aryl carbonyl, alkoxy carbonyl, aryloxy carbonyl, and aminocarbonyl.

The aryl groups and the aryl portion of the aryl carbonyl and aryloxy carbonyl groups preferably contain 6 to 10 carbon atoms (e.g., phenyl, naphthyl) and include substituted and unsubstituted groups. Useful substituents include halogen, cyano, alkyl, carboxy, alkyl carbonyl, aryl carbonyl, alkoxy carbonyl, aryloxy carbonyl, and aminocarbonyl.

Useful cations include organic and inorganic cations, such as a proton, an onium ion (e.g., ammonium, sulfonium, alkyl ammonium, aryl ammonium, alkyl sulfonium, aryl sulfonium), an alkali metal ion from Group IA of the Periodic Table (e.g., sodium, potassium), an alkaline earth metal ion from Group IIA of the Periodic Table (e.g., calcium) and a metal ion from Group IB, IIB and IVA of the Periodic Table (e.g., silver, zinc, cadmium, lead). (The periodic table referred to herein is that

shown on page 628 of Webster's Seventh New Collegiate Dictionary, G & C Merriam Company, Springfield, Mass., 1969.

While the Formula I compounds are depicted as mercaptides it is contemplated that the analogous selenium and tellurium compounds would be useful as latent image stabilizers.

Another embodiment of this invention is a photographic silver halide emulsion containing a latent image stabilizing amount of a compound as described above.

Yet another embodiment of this invention is a photographic element comprising a support bearing a layer of a silver halide emulsion containing a latent image stabilizing amount of a compound as described above.

Still another embodiment of this invention is a process of stabilizing a photographic silver halide emulsion against fading of the silver halide latent image between imagewise exposure and development of a visible image, comprising adding to the emulsion a latent image stabilizing amount of compound as described above.

Particularly preferred compounds according to the present invention are those having the structural formula I above wherein:

$R^1$  is alkyl of 1 to 4 carbon atoms;

$R^2$  and  $R^3$  are each hydrogen;

$R^4$  and  $R^5$  are each individually hydrogen or alkyl of 1 to 4 carbon atoms; and

$M^{\oplus n}$  is a monovalent cation from Group IA to IB of the Periodic Table.

Exemplary compounds according to the present invention are tabulated below.

TABLE I

| No. | $M^{\oplus n}$           | $R_1$  | $R_2$ | $R_3$ | $R_4$        | $R_5$           |
|-----|--------------------------|--------|-------|-------|--------------|-----------------|
| 1   | $Na^{\oplus}$            | H      | H     | H     | H            | H               |
| 2   | $Ag^{\oplus}$            | H      | H     | H     | H            | H               |
| 3   | $Na^{\oplus}$            | $CH_3$ | H     | H     | H            | $CH_3$          |
| 4   | $Ag^{\oplus}$            | $CH_3$ | H     | H     | H            | $CH_3$          |
| 5   | $Na^{\oplus}$            | H      | H     | H     | H            | $CH_3$          |
| 6   | $K^{\oplus}$             | $CH_3$ | H     | H     | H            | $C_6H_5$        |
| 7   | $Na^{\oplus}$            | $CH_3$ | H     | H     | H            | CN              |
| 8   | $Na^{\oplus}$            | $CH_3$ | H     | H     | H            | $COOC_2H_5$     |
| 9   | $Na^{\oplus}$            | $CH_3$ | H     | H     | H            | $CONH_2$        |
| 10  | $Na^{\oplus}$            | $CH_3$ | Br    | H     | H            | $CH_3$          |
| 11  | $Na^{\oplus}$            | H      | H     | H     | $CO_2C_2H_5$ | $CO_2C_2H_5$    |
| 12  | $Na^{\oplus}$            | $CH_3$ | H     | H     | $CO_2C_2H_5$ | $CO_2C_2H_5$    |
| 13  | $Na^{\oplus}$            | $CH_3$ | H     | H     | $CO_2C_2H_5$ | $-C_6H_5$       |
| 14  | $Na^{\oplus}$            | $CH_3$ | H     | H     | H            | $-C_6H_4SO_3-p$ |
| 15  | $^{+}Pb^{\oplus \oplus}$ | $CH_3$ | H     | H     | H            | $CH_3$          |
| 16  | $^{+}Zn^{\oplus \oplus}$ | $CH_3$ | H     | H     | H            | $CH_3$          |
| 17  | $^{+}Cd^{\oplus \oplus}$ | $CH_3$ | H     | H     | H            | $CH_3$          |

Compounds of the present invention can be prepared by hydrolyzing the corresponding N-alkenyl thiazolium salt in an aqueous or dilute gelatin solution using an appropriate base, such as sodium hydroxide, and, if necessary, performing a cation exchange reaction using an aqueous solution of a suitable salt, such as a nitrate, of the desired cation. These procedures are analogous to those reported by W. H. Mills, et al., J. Chem. Soc., 123, 2353 (1923) and R. R. Williams and A. E. Ruehle, J. Amer. Chem. Soc., 57, 1856-76 (1935).

The N-alkenyl thiazolium salts can be prepared by reacting the corresponding thiazole with an appropriate alkenyl halide.

The silver halide emulsions employed in the present invention can be any of the silver halide emulsions known in the art which are desirably protected against latent image fading. The silver halide emulsions can be comprised of silver bromide, silver chloride, silver chlorobromide, silver chloroiodide, silver bromoiodide, silver chlorobromoiodide or mixtures thereof. The emulsions can include coarse, medium or fine grain silver halide grains and can be monodisperse or polydisperse.

The silver halide emulsions are preferably negative-working emulsions. They can be chemically sensitized with active gelatin, as illustrated by T. H. James, *The Theory of the Photographic Process*, 4th Ed., Macmillan, 1977, pp. 67-76, or with sulfur, selenium, tellurium, gold, platinum, palladium, iridium, osmium, rhenium or phosphorus sensitizers or combinations of these sensitizers, such as at pAg levels of from 5 to 10, pH levels of from 5 to 8 and temperatures of from 30° to 80° C., as illustrated by *Research Disclosure*, Vol 134, June 1975, Item 13452, Sheppard et al. U.S. Pat. No. 1,623,499, Matthies et al. U.S. Pat. No. 1,673,522, Waller et al. U.S. Pat. No. 2,399,083, Damschroder et al. U.S. Pat. No. 2,642,361, McVeigh U.S. Pat. No. 3,297,447, Dunn U.S. Pat. No. 3,297,446, McBride U.K. Pat. No. 1,315,755, Berry et al. U.S. Pat. No. 3,772,031, Gilman et al. U.S. Pat. No. 3,761,267, Ohi et al. U.S. Pat. No. 3,857,711, Klinger et al. U.S. Pat. No. 3,565,633, Oftedahl U.S. Pat. Nos. 3,901,714 and 3,904,415 and Simons U.K. Pat. No. 1,395,696; chemical sensitization being optionally conducted in the presence of thiocyanate derivatives, as described in Neitz et al. U.S. Pat. No. 2,222,264, Damschroder U.S. Pat. No. 2,642,361; thioether compounds, as disclosed in Lowe et al. U.S. Pat. No. 2,521,926, Williams et al. U.S. Pat. No. 3,021,215 and Bigelow U.S. Pat. No. 4,054,457 and azaindenes, azapyridazines and azapyrimidines, as described in Dostes U.S. Pat. No. 3,411,914, Kuwabara et al. U.S. Pat. No. 3,554,757, Oguchi et al. U.S. Pat. No. 3,565,631 and Oftedahl U.S. Pat. No. 3,901,714. Additionally or alternatively, the emulsions can be reduction sensitized e.g., with hydrogen, as illustrated by Janusonis U.S. Pat. No. 3,891,446 and Babcock et al. U.S. Pat. No. 3,984,249, by low pAg (e.g., less than 5) high pH (e.g., greater than 8) treatment or through the use of reducing agents, such as stannous chloride, thiourea dioxide, polyamines and amineboranes, as illustrated by Allen et al. U.S. Pat. No. 2,983,609, Oftedahl et al. *Research Disclosure*, Vol. 136, August 1975, Item 13654, Lowe et al. U.S. Pat. Nos. 2,518,696 and 2,739,060, Roberts et al. U.S. Pat. Nos. 2,743,182 and 2,743,183, Chambers et al. U.S. Pat. No. 3,026,203 and Bigelow et al. U.S. Pat. No. 3,361,564. (*Research Disclosure* is published by Industrial Opportunities Ltd., Homewell, Havant Hampshire, PO9 1EF, United Kingdom.)

The silver halide emulsions can be spectrally sensitized with dyes from a variety of classes, including the polymethine dye class, which includes the cyanines, merocyanines, complex cyanines and merocyanines (i.e., tri-, tetra-, and poly-nuclear cyanines and merocyanines), oxonols, hemioxonols, styryls, merostyryls and streptocyanines. Particularly useful dyes are benzoxazole, benzimidazole and benzothiazole carbocyanine dyes.

The photographic silver halide emulsions can contain various colloids alone or in combination as vehicles. Suitable hydrophilic material include both naturally occurring substances such as proteins, protein derivatives, cellulose derivatives, e.g., cellulose esters, gelatin e.g., alkali-treated gelatin (cattle, bone or hide gelatin) or acid-treated gelatin (pigskin gelatin), gelatin derivatives e.g., acetylated gelatin, phthalated gelatin and the like, polysaccharides such as dextran, gum arabic, zein, casein, pectin, collagen derivatives, collodion, agar-agar, arrowroot, albumin and the like. The vehicles can be hardened by conventional procedures. Further details of the vehicles and hardeners are provided in *Research Disclosure*, December 1978, Item 17643, Sections IX and X.

The latent image stabilizing compound can be added to the silver halide emulsions at any point subsequent to precipitation of the silver halide grains so that it will interact with the silver halide grains prior to exposure of the emulsion. Preferably, the latent image stabilizing compound is added to the emulsion after chemical and spectral sensitization, but prior to coating. However, it can be present during these sensitization processes.

The optimum amount of latent image stabilizing compound added to the emulsion will depend upon such factors as the particular latent image stabilizing compound, the particular silver halide emulsion, the location of latent image formation, the nature of other components of the emulsion, and the like. Useful amounts are generally within the range 0.005 to 10 millimoles of latent image stabilizer per mole of silver. Preferably, the latent image stabilizing compound is incorporated in the emulsion in an amount of 0.05 to 10 millimoles of latent image stabilizer per mole of silver.

The photographic silver halide emulsions of this invention and photographic elements employing them can contain other addenda conventional in the photographic art. Useful addenda are described, for example, in *Research Disclosure*, December 1978, Item 17643. Useful addenda include spectral sensitizing dyes and desensitizers, antifoggants, couplers (such as dye forming couplers, masking couplers and DIR couplers) DIR compounds, anti-strain agents, image dye stabilizers, absorbing materials such as filter dyes and UV absorbers, light scattering materials, coating aids, plasticizers and lubricants, and the like.

The photographic elements of the present invention can be simple black-and-white or monochrome elements comprising a support bearing a layer of the silver halide emulsion, or they can be multilayer and/or multi-color elements. They can be designed for processing with separate solution or for in camera processing. Multicolor elements contain dye image forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsion or emulsions can be disposed as one or more segmented layers, e.g., as by the use of microvessels or microcells, as described in Whitmore U.S. patent application Ser. No. 184,714 filed Sept. 9, 1980.

Sept. 9, 1968. A preferred color photographic element according to 65 this invention comprises a support bearing at least one blue-sensitive silver halide emulsion layer having associated therewith a yellow dye-forming coupler, at least

one green-sensitive silver halide emulsion layer having associated therewith a magenta dye-forming coupler and at least one red-sensitive silver halide emulsion layer having associated therewith a cyan dye-forming 5 coupler, at least one of the silver halide emulsion layers containing a latent image stabilizing compound of this invention. In accordance with a particularly preferred aspect of the present invention, the latent image stabilizing compound is contained in a yellow dye-forming 10 blue-sensitive silver halide emulsion.

The elements of the present invention can contain additional layers conventional in photographic elements, such as overcoat layers, spacer layers, filter layers, antihalation layers, scavenger layers and the like.

15 The support can be any suitable support used with photographic elements. Typical supports include polymeric films, paper (including polymer-coated paper), glass and the like. Details regarding supports and other layers  
20 of the photographic elements of this invention are contained in *Research Disclosure*, December 1978, Item 17643, referred to above, the disclosure of which is incorporated herein by reference.

The following examples further illustrate this invention.

### PREPARATIVE EXAMPLE 1

### 3-Allyl-2,4-dimethylthiazolium bromide (Comparative Compound)

This compound was prepared as follows:

2,4-Dimethylthiazole (6.04 g, 0.05 mole), 3-bromopropene (6.6 g, 0.055 mole) and butyronitrile (25 ml) were combined and refluxed for 2 hours. Upon cooling a brown oil solidified into a wet ivory powder (8.15 g) which was collected by filtration. The powder was dissolved in methanol, combined with aqueous potassium bromide to make the bromide salt, treated with decolorizing charcoal and filtered while hot. The filtrate was poured into ethyl ether to force the bromide salt out of solution as an oil. The ethyl ether was decanted and the oil which remained was chilled in a dry ice/acetone bath, filtered and dried at 60° to yield 3.86 g (33%) of the title compound as a solid; m.p. 130° C.

### PREPARATIVE EXAMPLE 2

### The soluble mercaptide of the structure



was prepared as follows:

An aqueous solution of the product of Preparative Example 1 (6.4 mmoles) was hydrolyzed at 24° C. with two equivalents of 1 molar sodium hydroxide (pH ~ 11.5) to yield 6.4 mmoles of the desired product. At this temperature and alkalinity it took less than two minutes to convert the thiazolium salt to the colorless, water-soluble sodium mercaptide.

### PREPARATIVE EXAMPLE 3

The sparingly soluble silver mercaptide of the structure:



was prepared by the following procedure:

1. Distilled water (50 ml), deionized bone gelatin (500 mg) and 3-allyl-2,4-dimethylthiazolium hexafluorophosphate were combined at 50° C./pH 5.3 pAg 9.1.

2. The solution was adjusted to pH 11.3 (pAg 13.5) by adding 1 molar sodium hydroxide solution (~40 drops). 15

3. The sodium mercaptide was converted to a small-particle dispersion of the silver mercaptide by adding aqueous silver nitrate (26.9 mg AgNO<sub>3</sub>/10 ml H<sub>2</sub>O) with vigorous stirring (pH 11.2/pAg 12.5).

4. The pH was lowered to 7.0 with 1 normal nitric acid. 20

### EXAMPLE 1

A series of photographic silver halide coatings were prepared as follows:

10 coatings were tested using three different procedures as follows:

A. Exposed through a step tablet for 1/25 second to a 500 watt, 2850° K. tungsten light and immediately processed for 6 minutes in a p-methylaminophenol sulfate/hydroquinone developer, fixed, washed and dried.

B. Stored for one week at 48.9° C. and 50% relative humidity and then exposed and processed as in (A).

C. Exposed as in (A), stored for one week as in (B) and then processed as in (A).

The relative speeds obtained with the coatings using each of the three procedures are shown in Table II, which follows. Procedure (C) shows the effect of latent image fading relative to both procedures (A) and (B). The greater the loss of relative speed, the greater the amount of latent image fading.

TABLE II

| Coating        | Compound                                                                            | Amount<br>(mmoles/mole Ag) | Relative Speed <sup>1</sup> |     |      |
|----------------|-------------------------------------------------------------------------------------|----------------------------|-----------------------------|-----|------|
|                |                                                                                     |                            | A                           | B   | C    |
| 1 (control)    | None                                                                                | —                          | 100                         | 102 | 15.9 |
| 2 (comparison) |  | 3.2                        | 95                          | 107 | 16.5 |
| 3 (comparison) |  | 6.4                        | 97                          | 138 | 18.5 |
| 4 (invention)  |  | 3.2                        | 141                         | 141 | 174  |
| 5 (invention)  |  | 6.4                        | 102                         | 91  | 112  |
| 6 (comparison) |  | 3.2                        | 107                         | 110 | 29.5 |

TABLE II-continued

| Coating        | Compound                                                                                                                                | Amount<br>(mmoles/mole Ag) | Relative Speed <sup>1</sup> |    |    |
|----------------|-----------------------------------------------------------------------------------------------------------------------------------------|----------------------------|-----------------------------|----|----|
|                |                                                                                                                                         |                            | A                           | B  | C  |
| 7 (comparison) | $\text{CH}_3 \text{---} \text{CH}=\text{CH} \text{---} \text{N}(\text{CH}_3)_2 \text{---} \text{S}^\oplus \text{---} \text{Na}^\ominus$ | 6.4                        | 54                          | 53 | 18 |

<sup>1</sup> Speed was measured relative to coating 1 tested by procedure A.

These data show that only with an inventive compound (Coatings 4 and 5) was latent image fading prevented or significantly minimized. The thiazole salt from which the inventive compound was derived (Coatings 2 and 3) and an acyclic comparison compound with an N-alkyl substituent (Coatings 6 and 7) had almost as much latent image fading as the control (Coating 1).

### EXAMPLES 2-10

Compounds 1, 3, 5, 7, 8 and 9 from Table I were tested as described in Example 1 except that the emulsion was coated at pH 5.4 and pAg 8.9. Table III lists the sensitometric results.

TABLE III

| Example | Compound | mmoles/mole Ag | Relative Speed |      |     |
|---------|----------|----------------|----------------|------|-----|
|         |          |                | A              | B    | C   |
| 2       | None     | —              | 100            | 82   | 5.7 |
| 3       | 1        | 0.02           | 204            | 204  | 129 |
| 4       | 3        | 1.50           | 174            | 170  | 200 |
| 5       | 5        | 1.50           | 174            | 148  | 174 |
| 6       | 7        | 1.50           | 47             | 24.5 | 8.5 |
| 7       | 8        | 1.50           | 74             | 69   | 29  |
| 8       | 9        | 1.0            | 151            | 145  | 58  |
| 9       | None     | —              | 100            | 91   | 67  |
| 10      | 7        | 0.1            | 110            | 95   | 83  |

### EXAMPLES 11-17

Compounds 3, 4, 15, 16 and 17 from Table I and the comparison compound from coatings 2 and 3 of Example 1 were tested as described in Example 1 except that exposure was for 1/50 second with a 500 watt 5500° K. light source. The sensitometric results are reported in Table IV below.

TABLE IV

| Example | Compound   | mmoles/mole Ag | Relative Speed |     |     |
|---------|------------|----------------|----------------|-----|-----|
|         |            |                | A              | B   | C   |
| 11      | None       | —              | 100            | 166 | 50  |
| 12      | Comparison | 3.0            | 97             | 204 | 49  |
| 13      | 3          | 3.0            | 148            | 110 | 148 |
| 14      | 4          | 3.0            | 123            | 105 | 95  |
| 15      | 15         | 3.0            | 132            | 102 | 126 |
| 16      | 16         | 3.0            | 145            | 112 | 148 |
| 17      | 17         | 3.0            | 123            | 110 | 118 |

### EXAMPLE 18

A first photographic element (Element 1) was prepared having the following pertinent structure:

| Overcoat:                                                                                                                                                                    |
|------------------------------------------------------------------------------------------------------------------------------------------------------------------------------|
| Blue-Sensitive Silver Halide Emulsion                                                                                                                                        |
| Layer:                                                                                                                                                                       |
| 0.80 $\mu\text{m}$ sulfur + gold sensitized AgBr emulsion (1.62 g Ag/m <sup>2</sup> ); gelatin (1.72 g/m <sup>2</sup> ); yellow dye forming coupler (0.33 g/m <sup>2</sup> ) |

-continued

| Overcoat                                                                                                                                                                       |
|--------------------------------------------------------------------------------------------------------------------------------------------------------------------------------|
| Blue-Sensitive Silver Halide Emulsion                                                                                                                                          |
| Layer:                                                                                                                                                                         |
| 0.80 $\mu\text{m}$ sulfur + gold sensitized AgBr emulsion (0.78 g Ag/m <sup>2</sup> ) + gelatin (1.25 g/m <sup>2</sup> ) + yellow dye-forming coupler (0.86 g/m <sup>2</sup> ) |
| Yellow Filter Layer                                                                                                                                                            |
| Green-Sensitive Silver Halide Emulsion                                                                                                                                         |
| Layer                                                                                                                                                                          |
| Red-Sensitive Silver Halide Emulsion                                                                                                                                           |
| Layer                                                                                                                                                                          |
| Green-Sensitive Silver Halide Emulsion                                                                                                                                         |
| Layer                                                                                                                                                                          |
| Red-Sensitive Silver Halide Emulsion                                                                                                                                           |
| Layer                                                                                                                                                                          |
| Film Support                                                                                                                                                                   |

A second photographic element (Element 2) was prepared which was identical to the first element except that the blue-sensitive silver halide emulsion layer furthest from the support contained 0.18 mmoles per mole of silver of the latent image stabilizer prepared in Preparative Example 3, i.e.



The two elements were tested according to the procedures described in Example 1, except that storage in procedures B and C was for 4 weeks at 25.6° C. and 50% relative humidity, and that processing was as described in British Journal of Photography, July 1974, pp. 579-589. The following results were obtained:

| Element       | Relative Speed <sup>1</sup> |     |    |
|---------------|-----------------------------|-----|----|
|               | A                           | B   | C  |
| 1 (control)   | 100                         | 91  | 60 |
| 2 (invention) | 102                         | 100 | 95 |

<sup>1</sup> Speed was measured relative to Element 1 tested by Procedure A.

These data show that the element according to the invention had significantly less latent image fading than the control element.

This invention has been described in detail with particular reference to preferred embodiments thereof but it will be understood that variations and modifications can be effected within the spirit and scope of the invention.

What is claimed is:

1. A photographic silver halide emulsion containing as a latent image stabilizer, in a latent image stabilizing amount, a compound represented by the formula:



5

wherein:

 $\text{R}^1$  is hydrogen, alkyl, or aryl; $\text{R}^2$  and  $\text{R}^3$  are each individually hydrogen, alkyl, alkoxy, carboxy, alkoxy carbonyl, or aminocarbonyl; $\text{R}^4$  and  $\text{R}^5$  are each individually hydrogen, alkyl, aryl, cyano, halogen, formyl, carboxy, alkyl carbonyl, aryl carbonyl, alkoxy carbonyl, aryloxy carbonyl or aminocarbonyl; $n$  is an integer of 1 or 2; and $\text{M}^{\oplus n}$  is a cation of valence  $n$ .

2. A photographic silver halide emulsion of claim 1

wherein:

 $\text{R}^1$  is alkyl of 1 to 4 carbon atoms; $\text{R}^2$  and  $\text{R}^3$  are each hydrogen; $\text{R}^4$  and  $\text{R}^5$  are each individually hydrogen or alkyl of 1 to 4 carbon atoms; and $\text{M}^{\oplus n}$  is a monovalent cation from Group IA or IB of the Periodic Table.

3. A photographic silver halide emulsion of claim 1

wherein the latent image stabilizing compound is represented by the structural formula:



35

wherein:

 $\text{M}^{\oplus}$  is a sodium or silver cation.

4. A photographic silver halide emulsion of claim 1, 2, or 3 wherein the latent image stabilizing compound is present in an amount of from 0.005 to 100 mmoles per mole of silver.

5. A photographic element comprising a support bearing a layer of a silver halide emulsion of any one of claims 1, 2 or 3.

6. A photographic element of claim 5 wherein the latent image stabilizing compound is present in an amount of from 0.005 to 100 mmoles per mole of silver.

7. A photographic element of claim 5 wherein the latent image stabilizing compound is present in an amount of from 0.05 to 10 mmoles per mole of silver.

8. In a color photographic element comprising a support bearing at least one blue-sensitive silver halide emulsion layer having associated therewith a yellow dye-forming coupler, at least one green-sensitive silver halide emulsion layer having associated therewith a magenta dye-forming coupler and at least one red-sensitive silver halide emulsion layer having associated therewith a cyan dye-forming coupler, the improvement wherein at least one of the silver halide emulsion layers contains as a latent image stabilizer, in a latent image stabilizing amount, a compound represented by the formula:

55

60

65



wherein:

 $\text{R}^1$  is hydrogen, alkyl, or aryl; $\text{R}^2$  and  $\text{R}^3$  are each individually hydrogen, alkyl, alkoxy, carboxy, alkoxy carbonyl, or aminocarbonyl; $\text{R}^4$  and  $\text{R}^5$  are each individually hydrogen, alkyl, aryl, cyano, halogen, formyl, carboxy, alkyl carbonyl, aryl carbonyl, alkoxy carbonyl, aryloxy carbonyl or aminocarbonyl; $n$  is an integer of 1 or 2; and $\text{M}^{\oplus n}$  is a cation of valence  $n$ .

9. A color photographic element of claim 8 wherein:

 $\text{R}^1$  is alkyl of 1 to 4 carbon atoms; $\text{R}^2$  and  $\text{R}^3$  are each hydrogen; $\text{R}^4$  and  $\text{R}^5$  are each individually hydrogen or alkyl of 1 to 4 carbon atoms; and $\text{M}^{\oplus n}$  is a monovalent cation from Group IA or IB of the Periodic Table.

10. In a color photographic element of claim 8 wherein the latent image stabilizing compound is represented by the structural formula:



wherein:

 $\text{M}^{\oplus}$  is a sodium or silver cation.

11. A color photographic element of any one of claims 8, 9 or 10 wherein the latent image stabilizing compound is contained in a blue-sensitive silver halide emulsion layer.

12. A color photographic element of any one of claims 8, 9 or 10 wherein the latent image stabilizing compound is present in an amount of from 0.05 to 10 mmoles per mole of silver.

13. A process of stabilizing a photographic silver halide emulsion against fading of the silver halide latent image between imagewise exposure and development of a visible image, comprising adding to the emulsion a latent image stabilizing amount of a compound represented by the formula:



wherein:

 $\text{R}^1$  is hydrogen, alkyl, or aryl; $\text{R}^2$  and  $\text{R}^3$  are each individually hydrogen, alkyl, alkoxy, carboxy, alkoxy carbonyl, or aminocarbonyl; $\text{R}^4$  and  $\text{R}^5$  are each individually hydrogen, alkyl, aryl, cyano, halogen, formyl, carboxy, alkoxy carbonyl, aryloxy carbonyl or aminocarbonyl;

n is an integer of 1 or 2; and  
 $M^{\oplus n}$  is a cation of valence n.

14. A process of claim 13 wherein the latent image stabilizing compound is added in an amount of from 0.005 to 100 mmoles per mole of silver.

15. A process of claim 13 wherein the latent image stabilizing compound is added following chemical and spectral sensitization.

16. A latent image stabilizing compound having the formula:



wherein:

R<sup>1</sup> is hydrogen, alkyl, or aryl;  
R<sup>2</sup> and R<sup>3</sup> are each individually hydrogen, alkyl, alkoxy, carboxy, alkoxy carbonyl, or aminocarbonyl;  
R<sup>4</sup> and R<sup>5</sup> are each individually hydrogen, alkyl, aryl, cyano, halogen, formyl, carboxy, alkyl carbonyl,

25

15

aryl carbonyl, alkoxy carbonyl, aryloxy carbonyl or aminocarbonyl;

n is an integer of 1 or 2; and  
 $M^{\oplus n}$  is a cation of valence n.

17. A latent image stabilizing compound of claim 16 wherein:

R<sup>1</sup> is alkyl of 1 to 4 carbon atoms;  
R<sup>2</sup> and R<sup>3</sup> are each hydrogen;  
R<sup>4</sup> and R<sup>5</sup> are each individually hydrogen or alkyl of 1 to 4 carbon atoms; and  
M<sup>⊕</sup> is a monovalent cation from Group IA or IB of the Periodic Table.

18. A latent image stabilizing compound having the formula:



wherein:

M<sup>⊕</sup> is a sodium or silver cation.

\* \* \* \* \*

30

35

40

45

50

55

60

65